# EUROPEAN PATENT SPECIFICATION

(11) **EP 0 699 458 B1**
(45) Date of publication and mention of the grant of the patent: **19.01.2000**
(21) Application number: 95113630.8
(22) Date of filing: 30.08.1995
(51) Int. Cl.: A63C 5/12

(54) **Process of fabricating safety strong ski**
Verfahren zur Herstellung eines starken und zuverlässigen Skis
Procédé de fabrication d'un ski solide et fiable

(30) Priority: 31.08.1994 JP 23070494; 05.10.1994 JP 26634194
(43) Date of publication of application: 06.03.1996
(73) Proprietor: Japana Co., Ltd., Nagoya 450-0002 (JP)
(72) Inventor: Fukushima, Toshiharu, Hamamatsu-shi, Shizuoka-ken (JP); Yasui, Takuo, Hamamatsu-shi, Shizuoka-ken (JP); Okada, Masuhiro, Hamamatsu-shi, Shizuoka-ken (JP); Suzuki, Katsunori, Hamamatsu-shi, Shizuoka-ken (JP)
(74) Representative: ffrench-Lynch, Cecil

(56) References cited:
- EP-A- 0 428 885
- AT-A- 296 105
- AT-A- 384 171
- DE-A- 3 545 455
- DE-A- 4 106 911

## Description

### FIELD OF THE INVENTION

This invention relates to a ski for sliding on snow and, more particularly, to a process of economically fabricating a safety strong ski.

### DESCRIPTION OF THE RELATED ART

A typical example of the process of fabricating a ski is disclosed in EP-A-0 428 885 (corresponding to JP-A-3182275 or FR-A-2 654 645).

According to the above publication which is represented in Figs. 1-3 of the drawings hereof, the prior art process starts with preparation of a split-type mold 1, component members of the ski, a expandable flexible tubular member 2, an upper reinforcing sheet member 3 of metal and a foamable material such as polyurethane foam. The component members are assembled into an upper structure 4a in a cavity of an upper mold half 5a and a lower structure 4b in a cavity of a lower mold half 5b. The lower structure 4b has a running surface 4c and sole edge members 4d, and will form a hollow space 6 together with the upper structure 4b upon assembly of the split-type mold.

Before the assembly, the expandable flexible tubular member 2 is placed on the lower structure 4b, and the upper reinforcing sheet member 3 is laminated on the expandable flexible tubular member 2.

The upper mold half 5a is assembled with the lower mold half 5b. Then, the hollow space 6 takes place between the upper structure 4a and the lower structure 4b, and the expandable flexible tubular member 2 and the upper reinforcing sheet member 3 are confined in the hollow space 6 as shown in figure 1A.

Subsequently, the polyurethane foam is injected into the expandable flexible tubular member 2, and the flexible tubular member 2 expands in the hollow space 6. The injection path is formed in the mold 1, and is usually located at one end portion in the longitudinal direction of the ski. The polyurethane foam (topographically) presses the flexible tubular member 2 directly against the inner surfaces of the upper/lower structures 4a/4b and through the upper reinforcing sheet member 3 against the upper structure 4a as shown in figure 1B. The polyurethane foam forms a core member 7 filling the space 6.

When the polyurethane foam is cured, the upper/lower mold halves 5a/5b are separated, and the ski is taken out from the mold 5a/5b.

The reinforcing sheet member 3 is replaceable with a reinforcing flexible sheet member 8 as shown in figure 2.

While an operator is assembling the upper structure 4a and the lower structure 4b, the mold halves 5a and 5b may be inverted as shown in figure 3, and prepregs 8a, 8b and 8c may be used as the reinforcing members. The prepregs 8a, 8b and 8c are covered into fiber-reinforced plastic resin layers through heat treatment.

However, the prior art process encounters a problem in that the strength of the core member 6 is not constant. This is because of the fact that the urethane foam does not uniformly spread over the inner space of the mold 1. Another reason for the insufficient strength is uncontrollable expansion of the flexible tubular member 2 in the mold 1. While the urethane foam is expanding in the flexible tubular member 2, the flexible tubular member 2 moves the reinforcing member 3, and changes the original relative location between the reinforcing member 3 and the mold 1. This results in a stress concentration and undesirable damage of the reinforcing member 3. If the upper and lower reinforcing members are the prepregs 8a, 8b and 8c, void tends to take place in the fiber-reinforced plastic resin layers, and deteriorates the ski.

Another problem inherent in the prior art process is the complicated mold 1 due to an injection path for the polyurethane foam, and the complicated mold 1 increases the production cost.

Yet another problem inherent in the prior art process is burs or residue of the polyurethane left around the injection hole of the ski and in the mold 1. The manufacturer is required to remove the burs from the mold and the ski, and the cleaning work and the elimination work further increases the production cost.

Another prior art process of fabricating a ski is disclosed in JP-A-1284272, and figure 4 illustrates a ski fabricated through the second prior art fabrication process.

According to the above mentioned JP-A-1 284 274, an upper structure 10a and a lower structure 10b are separately assembled. A core member 10c, an upper reinforcing member 10d of fiber-reinforced plastic resin laminated on the upper and side surfaces of the core member 10c and an inverted U-shaped surface member 10e encapsulating the upper reinforcing member 10d and the core member 10c form in combination the upper structure 10a. On the other hand, the lower structure 10b includes a lower reinforcing member 10f of fiber-reinforced plastic resin, a sliding plate member 10g attached to the lower surface of the lower reinforcing member 10f and sole edge members 10h attached to both sides of the sliding plate member 10g.

At least one of the upper and lower reinforcing members 10d and 10f is a laminations of bias sheets, and the reinforcing fibers of the bias sheets extend at 45 degrees and at -45 degrees with respect to the longitudinal direction of the ski. The bias sheets enhance the torsional rigidity of the ski.

The upper and lower structures 10a and 10b thus prepared are bonded in such a manner that the lower surface of the core member 10c is held in contact with the upper surface of the lower reinforcing member 10f.

The second prior art process may be free from the problems due to the injection of the polyurethane. However, a problem is encountered in the second fabrication process in that the upper structure is liable to be separated from the lower structure due to sharing force resulted from undesirable large bending during the sliding on snow. This is dangerous.

Regarding the prior art, attention is further drawn to DE-A-35 45 455 which is directed to a method for manufacturing thermoplastic bodies having a core, and more specifically, said document is directed to the manufacture of a surfboard.

In accordance with the present invention a method as set forth in claim 1 is provided. Preferred embodiments of the invention are disclosed in the dependent claims.

### SUMMARY OF THE INVENTION

It is therefore an important object of the present invention to provide a process which economically fabricate a safety strong ski.

To accomplish the object, the present invention proposes to internally produce foam from a foamable gum substance.

In accordance with the present invention, there is provided a process of fabricating a ski as set forth in claim 1. Preferred embodiments may be gathered from the dependent claims.

### BRIEF DESCRIPTION OF THE DRAWINGS

The features and advantages of the process of fabricating a ski according to the present invention will be more clearly understood from the following description taken in conjunction with the accompanying drawings in which:
Figs. 1A and 1B are cross sectional views showing the prior art process disclosed in EP-A-0 428 885;
Fig. 2 is a cross sectional view showing the alternative step of the prior art fabrication process;
Fig. 3 is a cross sectional view showing the alternative step of the prior art fabrication process;
Fig. 4 is a cross sectional view showing the ski fabricated through the prior art fabrication process disclosed in JP-A-1284272;
Fig. 5 is a cross sectional view showing the structure of a ski fabricated through a process according to the present invention;
Figs. 6A to 6C are cross sectional views showing a fabrication sequence of a process according to the present invention;
Fig. 7 is a cross sectional view showing a core structure incorporated in a ski fabricated through a first modification of the process described in conjunction with figures 6A to 6C;
Fig. 8 is a cross sectional view showing a core structure incorporated in a ski fabricated through a second modification;
Fig. 9 is a cross sectional view showing a core structure incorporated in a ski fabricated through a third modification;
Fig. 10 is a cross sectional view showing a core structure incorporated in a ski fabricated through a fourth modification;
Fig. 11 is a side view showing a core structure incorporated in a ski fabricated through a fifth modification;
Figs. 12A to 12D are schematic views showing modifications of a partition sheet;
Fig. 13 is a cross sectional view showing the structure of a ski fabricated through a process according to the present invention, however without showing the partition sheet;
Figs. 14A to 14D are views showing a process sequence for fabricating the ski shown in figure 13.

### DESCRIPTION OF THE PREFERRED EMBODIMENTS

### First Embodiment

Referring first to figure 5 of the drawings, a ski 20 fabricated through a process embodying the present invention comprises a generally inverted U-shaped surface member 21 defining an upper surface and side surfaces of the ski 20, and embosses 21a and 21b are formed in the upper portion of the surface member 21. The embosses 21a and 21b extend in a longitudinal direction of the ski 20. The surface member 21 is, by way of example, formed of polyamide elastomer, PET resin, ABS resin, polyvinyl chloride or ionomer.

The ski 20 further comprises a sliding surface member 22 providing a lower surface of the ski 20 and sole edge members 23a and 23b attached to both sides of the sliding surface member 22. The sliding surface member 22 is formed of polyethylene, and a skier presses the sliding surface member 22 to snow. The generally inverted U-shaped surface member 21 is terminated at both sides thereof at the sole edge members 23a and 23b, and is integral with the sole edge members 23a and 23b. The generally inverted U-shaped surface member 21, the sliding surface member 22 and the sole edge members 23a and 23b form an inner space.

The ski 20 further comprises a core member 24 formed from foamable substance, a partition sheet 25 snugly (topographically) enclosing the core member 24 and a reinforcing member 26 of fiber-reinforced plastic resin filling a gap between the inner surface of the generally inverted U-shaped surface member 21 and the core member 24.

The combined structure of the generally inverted U-surface member 21, the core member 24, the partition sheet 25 and the reinforcing member 26 is made from an upper structure 27 as will be described hereinlater. On the other hand, the sliding surface member 22 and the sole edge members 23a and 23b as a whole constitute a lower structure 28.

Description is hereinbelow made on the process embodying the present invention. The process starts with preparation of the members of the upper and lower structures 27 and 28 and a split-type mold 29. The split-type mold 29 is constituted by molding halves 29a and 29b, and the molding halves 29a and 29b are separated from one another for assembling the upper and lower structures 27 and 28 in cavities 29c/29d of the molding halves 29a/29b. Namely, an elongated piece 31 of foamable gum substance is partially wrapped in the partition sheet 25, and the elongated piece 31 of foamable gum substance and the partition sheet 25 is enclosed in a raw member 32 for the fiber-reinforced plastic resin. The partition sheet 25 is shorter than the periphery of the elongated piece 31 of foamable gum substance. In this instance, matrix fibers of the raw member 32 is in the same synthetic resin system as the foamable gum substance, and the adhesion is enhanced because of the concurrent thermo-set.

The term "foamable gum substance" means substance which is plastically deformable at room temperature and foamable at a temperature higher than the room temperature.

In this instance, the raw member 32 is shaped into a tubular configuration, and the tubular configuration enhances the torsional rigidity of the raw member 32. The tubular raw member 32 is formed from a lamination of non-set matrix fibers and reinforcing fibers or a prepreg where matrix resin is impregnated into reinforcing fibers. The matrix resin is, by way of example, formed of thermosetting synthetic resin such as, for example, epoxy, vinyl ester resin, polyester resin. Thermoplastic resin is also available for the matrix, and the non-set matrix may be in the form of pellet or powder. The reinforcing fibers are, by way of example, carbon fibers, glass fibers, aramid fibers or metallic fibers, these fibers may be selectively mixed.

The first example of the foamable gum substance is in the epoxy system, and contains 40 parts by weight of bisphenol A liquid epoxy resin, 60 parts by weight of bisphenol A solid epoxy resin, 10 parts by weight of setting agent such as, for example, dicyan-diamide, 8 parts by weight of setting promoter such as, for example, dichlorophenyl-dimethylurea and 30 parts by weight of foaming agent such as thermal expansion micro-capsules. The expansion ratio is regulated to 8.

The second example of the foamable gum substance is in the epoxy system, and contains 50 parts by weight of bisphenol A liquid epoxy resin, 50 parts by weight of bisphenol A solid epoxy resin, 18 parts by weight of setting agent, i.e., 8 parts by weight of amine adduct and 10 parts by weight of dicyandiamide (DICY) and 8 parts by weight of foaming agent such as, for example, hydroxybenzenesulfonilhydrazide (OBSH). The expansion ratio is regulated to 8. The second example may further contain 8 parts by weight of foaming promoter in urea system so as to lower the foaming temperature, and 5 parts by weight of protecting agent such as, for example, barium stearate or polysiloxane bonded to organic functional group so as to prevent cells from breakage during the foaming stage.

The third example of the foamable gum substance is the epoxy system, and contains 100 parts by weight of bisphenol A liquid epoxy resin, 20 parts by weight of latent low-temperature setting agent such as amine adduct and 8 parts of foaming agent such as, for example, hydroxybenzenesulfonilhydrazide (OBSH). The foaming is carried out around 80 degrees centigrade for 10 minutes, and, thereafter, the foam is cooled. The expansion ratio is regulated to 8. The third example may further contain 8 parts by weight of foaming promoter in urea system so as to lower the foaming temperature.

The fourth example of the foamable gum substance is in the polyester system, and contains 100 parts by weight of unsaturated polyester resin, 20 parts by weight of setting catalyst such as peroxide, 30 parts by weight of thermally expanding micro-capsules and 3 parts of viscosity increaser such as, for example, calcium hydroxide. The expansion ratio is also regulated to 8.

Glass balloon, ceramic balloon or phenol balloon may be added to the first to fourth examples of the foamable gum substance so as to increase the volume of the elongated piece 31 of foamable gum substance. When the balloon is added, the density of foamable gum substance is preferably regulated to 0.65. The amount of foamable gum substance in the cavity 29c is regulated in such a manner as to generate pressure ranging from 8 kg/cm² to 10 kg/cm².

The partition sheet 25 is, by way of example, formed of valcanized gum, elastomer in urethane system, elastomer in ester system or elastomer in polyamide system. The gum or the elastomer is required to be not less than 100 percent in elongation percentage before break, not less than 10 MPa in tensile strength, not less than 130 degrees centigrade in fusion point and 0.05 to 0.40 millimeter in thickness. If a substance has the elongation percentage not less than 200 percent and the tensile strength not less than 20 MPa, the substance is more preferable.

On the other hand, the sole edge members 23a/23b are assembled with the sliding surface member 22 in the cavity of the molding half 29b. The resultant structure at the assembling stage is illustrated in figure 6A.

Subsequently, the molding halves 29a and 29b are assembled, and the upper and lower structures 27 and 28 are confined in an inner space formed by the cavities 29c and 29d as shown in figure 6C.

The mold 29 is heated to 120 degrees centigrade, and is maintained for 35 minutes. Then, the heat foams the gum substance, and converts the raw member 32 to the reinforcing member 26 of fiber-reinforced plastic resin. While the foam is expanding in the inner space of the mold 29, the partition sheet 25 and the raw member 32 are outwardly moved, and are pressed to the inner surface of the surface member 21. Therefore, the reinforcing member 26 is snugly disposed (or topographical) along the inner surface of the surface member 21, and the reinforcing member 26, the partition sheet 25 and the core member 24 fill the inner space among the surface member 21, the sliding surface member 22 and the sole edge members 23a/23b.

The elongated piece 31 of foamable gum substance occupies the inner space among the surface member 21, the sliding surface member 22 and the sole edge members 23a and 23b, and uniformly supplies the foam. As a result, a void hardly takes place in the core member 24, and the core member 24 provides uniform strength along the longitudinal direction. Moreover, the air in the cavities is evacuated through abutting surfaces of the molding halves 29a and 29b before the foaming, because the raw member 32 encloses the elongated piece 31 of foamable gum substance. The partition sheet 25 causes the reinforcing member 26 to be closely held in contact with the inner surface of the surface member 21, and the matrix of the reinforcing member 26 is merged with the core member 24 because of the same synthetic resin system.

An injection hole and a vent are not necessary, and the mold 29 is simpler than the mold 1. The economical mold decreases the production cost of the ski 20.

The surface member 21 is integrated with the lower structure 28 during the heat treatment, and is never separated from the lower structure 28 during the skiing.

When 35 minutes pass, the foam is thermally set, and is converted to the core member 24. The core member 24, the partition sheet 25 and the reinforcing member 26 snugly fill the inner space of the mold 29, and the surface member 21 is integrated with the lower structure 28. The mold 29 is cooled by using water at 15 degrees centigrade for 10 minutes, and reaches room temperature equal to or less than 30 degrees centigrade. The ski 20 is completed in the mold 29 as shown in figure 6C, and the molding halves 29a and 29b are separated so as to take out the ski 20 from the mold 29.

The foam is internally produced in the mold 29, and the ski 20 is free from a burr due to the injection. A grinding stage for the burr is not necessary, and the production cost is further decreased.

As will be understood from the foregoing description, the foam uniformly generated from the gum substance eliminates a void from the core member 24, and the ski 20 is stronger than the prior art ski. The gum substance is exactly placed in the mode, and, accordingly, the foam uniformly presses the other components such as the raw member 32 to the inner surface of the surface member 21 and the sliding surface member 22 without undesirable movement. This feature further enhances the strength of the ski. The mold is simple, and no additional work is necessary for a burr. This results in reduction of the production cost. The ski 20 integrated in the mold 29 is free from undesirable separation, and is safe.

Various modifications are described as follows. First, two kinds of foamable gum substance may be used for two-layered core member structure made from a laminated structure 41a/41b of foamable gum substance. The core members are different in compressive rigidity. A lower elongated piece 41b of foamable gum produces foam for the hard core member, and an upper elongated piece 41a of foamable gum generates foam for the soft core member. The hard core member maintains a smooth sliding surface, and the soft core member takes up the shock from the snow ground to the skier.

Figure 8 illustrates a second modification, and a core structure is constituted by soft and hard core members arranged in parallel. The soft core member is made from an elongated piece 42a of first kind of foamable gum substance, and occupies the outside of the ski. On the other hand, the hard core member is made from an elongated piece 42b of second kind of foamable gum substance, and occupies the inside of the ski. The ski equipped provides a sharp inside edging and a soft outside edging to a skier.

Figure 9 illustrates a third modification, and a hard core member is sandwiched between soft core members. The hard core member is made from an elongated piece 43a of first kind of foamable gum substance, and the soft core members are made from elongated pieces 43b and 43c of second kind of foamable gum substance. The hard core member maintains a smooth sliding surface, and the soft core members provides the soft inside/outside edging to a skier.

Figure 10 illustrates a fourth modification, and a soft core member is wrapped by a hard core member. The soft core member is made from an elongated piece of second kind of foamable gum substance, and the hard core member is made from an elongated tube 44b of first kind of foamable gum substance. The hard core member maintains a smooth sliding surface, and the soft core member makes the ski light.

Figure 11 illustrates a fifth modification, and soft core members are merged with the front end portion and the rear end portion of a hard core member. The hard core member is made from an elongated piece 45a of first kind of foamable gum substance, and the soft core members are made from elongated pieces 45b and 45c of second kind of foamable gum substance. The soft core members provide easily deformable front and rear end portions to the ski, and makes the ski light. On the other hand, the hard core member in the central portion of the ski improves the durability of the ski. The soft core members contiguous to the hard core member change the flex pattern of the ski.

If the expansion ratio or the blending ratio of the foaming agent is differently regulated, the foaming gum substance is converted to both soft and hard core members, and the soft and hard core members are different in compressive rigidity.

Thus, the soft and hard core members allows the manufacturer to arbitrarily regulate the characteristics of the ski.

Although the partition sheet 25 partially wraps the elongated piece 31 of foamable gum substance except for the central area of the bottom surface, various modifications are employable as shown in figures 12A to 12D.

In detail, figure 12A shows the first modification 46a of the partition sheet 25. The first modification 46a extends on the upper surface of the elongated piece 31, and both side portions covers both upper corners 31a and 31b of the elongated piece 31.

The second modification is implemented by two parts 46. One of the two parts 46 extends from the upper corner 31a through the left side surface to the lower corner 31c, and the other part 46 covers the other upper corner 46b, the right side surface and the lower corner 31d.

The third modification 46c simply covers the upper surface of the elongated piece 31 of foamable gum substance.

The fourth modification is implemented by three parts 46d. The first part 46d is similar to the first modification 46a, and the second and third parts 46d covers the lower corners 31c and 31d.

In the first embodiment, the raw member 32 is shaped into a tubular configuration. There are various modifications of the raw member 32 for the fiber-reinforced plastic resin. The first modification of the raw member 32 is a flexible sheet, and the flexible sheet is wound on the entire surface of the elongated piece 31. In this modification, it is recommendable to use matrix fibers of the flexible sheet formed of the same synthetic resin system such as, for example, epoxy resin system as the foamable synthetic resin, because the flexible sheet is thermally set concurrently to the foam made from the elongated piece 31, thereby enhancing the adhesion between the reinforcing member 26 and the partition sheet 25.

### Second Embodiment

Figure 13 illustrates the structure of a ski fabricated through a process embodying the present invention however without showing the partition sheet. The ski largely comprises an upper structure 51 and a lower structure 52, and the upper structure 51 is integral with the lower structure 52.

The upper structure 51 includes a surface member 51a shaped into a generally inverted U-configuration, a reinforcing member 51b of fiber-reinforced plastic resin and a core member 51c of foam plastic resin. The reinforcing member 51b is closely held in contact with the inner surface of the surface member 51a, and the core member 51c is snugly received in an inner space of the reinforcing member 51b.

The lower structure 52 includes a sliding surface member 52a and sole edge members 52b and 52c attached to both sides of the sliding surface member 52a. The bottom surface of the sliding surface portion 52a is pressed against snow, and slides on the snow ground. The sliding surface member 52a is formed of high molecular polyethylene resin, and the polyethylene resin tends to be deformed over 120 degrees centigrade.

The lower portion of the reinforcing member 51b is fixed to the upper surface of the sliding surface member 52a, and the side portions of the surface member 51a are fixed to the upper surfaces of the sole edge members 52b and 52c, respectively. Thus, the upper structure 51 is integrated with the lower structure 52.

The process sequence is described hereinbelow with reference to figures 14A to 14D. The process starts with preparation of a mold 53, the surface member 51a, an elongated piece 55 of foamable gum substance, a flexible matrix sheet 55a, a tubular fabric member 55b made from reinforcing fibers, the sliding surface member 52a and sole edge members 52b and 52c. The foamable gum substance is plastically deformable at room temperature, and heat foams the foamable gum substance. The tubular fabric member 55b may contain reinforcing fibers woven into a tube. In this instance, the flexible matrix sheet 55a and the tubular fabric member 55b form in combination a raw member 55 for the reinforcing member 51c.

The surface member 51a is, by way of example, formed of polyamide elastomer, PET resin, ABS resin, polyvinyl chloride or ionomer.

The matrix resin is thermo-setting synthetic resin good in tack and drape at room temperature, and viscosity is preferably 10,000 cp at 60 degrees centigrade and hundreds cp at 110-120 degrees centigrade. Nylon and polycarbonate are not available, because they are solid at 120 degrees centigrade.

Although the reinforcing fibers are woven into the tube of the tubular fabric member 55b, a non-woven fabric is available, and the configuration is not limited to the tube. The reinforcing fibers are, by way of example, carbon fibers, glass fibers, aramid fibers or metallic fibers, or these fibers may be selectively mixed.

The first example of the foamable gum substance is in the epoxy system, and contains 50 parts by weight of bisphenol A liquid epoxy resin, 60 parts by weight of bisphenol A solid epoxy resin, 10 parts by weight of setting agent such as, for example, dicyan-diamide, 8 parts by weight of setting promoter such as, for example, dichlorophenyl-dimethylurea and 30 parts by weight of foaming agent such as thermal expansion micro-capsules. The expansion ratio is regulated to 8.

The second example of the foamable gum substance is in the epoxy system, and contains 50 parts by weight of bisphenol A liquid epoxy resin, 50 parts by weight of bisphenol A solid epoxy resin, 18 parts by weight of setting agent, i.e., 8 parts by weight of amine adduct and 10 parts by weight of dicyandiamide (DICY) and 8 parts by weight of foaming agent such as, for example, hydroxybenzenesulfonilhydrazide (OBSH). The expansion ratio is regulated to 8. The second example may further contain 8 parts by weight of foaming promoter in urea system so as to lower the foaming temperature, and 5 parts by weight of protecting agent such as, for example, barium stearate or polysiloxane bonded to organic functional group so as to prevent cells from breakage during the foaming stage.

The third example of the foamable gum substance is the epoxy system, and contains 100 parts by weight of bisphenol A liquid epoxy resin, 20 parts by weight of latent low-temperature setting agent such as amine adduct and 8 parts of foaming agent such as, for example, hydroxybenzenesulfonilhydrazide (OBSH). The foaming is carried out around 80 degrees centigrade for 10 minutes, and, thereafter, the foam is cooled. The expansion ratio is regulated to 8. The third example may further contain 8 parts by weight of foaming promoter in urea system so as to lower the foaming temperature.

The fourth example of the foamable gum substance is in the polyester system, and contains 100 parts by weight of unsaturated polyester resin, 20 parts by weight of setting catalyst such as peroxide, 30 parts by weight of thermally expanding micro-capsules and 3 parts of viscosity increaser such as, for example, calcium hydroxide. The expansion ratio is also regulated to 8.

Glass balloon, ceramic balloon or phenol balloon may be added to the first to fourth examples of the foamable gum substance so as to increase the volume of the elongated piece 54 of foamable gum substance. When the balloon is added, the density of foamable gum substance is preferably regulated to 0.65. The amount of foamable gum substance in the cavity 53c is regulated in such a manner as to generate pressure ranging from 8 kg/cm² to 10 kg/cm².

The elongated piece 54 of foamable gum substance is inserted into an inner space of the tubular fabric member 55b, and the flexible matrix sheet 55a is wound on the tubular fabric member 55b as shown in figure 14A.

Subsequently, the surface member 51a, the flexible matrix sheet 55a and the tubular fabric member 55b laminated on the elongated piece 54, the sliding surface member 52a and the sole edge members 52b and 52c are assembled in the mold 53 as shown in figure 14B.

The mold 53 is a split-type, and molding halves 53a and 53b constitute the split-type mold 53. The molding half 53a has a cavity 53c corresponding to the outer configulation of the upper structure 51, and a cavity 53d in the other molding half 53b corresponds to the outer configuration of the lower structure 52. The surface member 51a is inserted into the cavity 53c, and the flexible matrix sheet 55a and the tubular fabric member 55b wound on the elongated piece 54 is put on the inner surface of the surface member 51a. On the other hand, the sliding surface member 52a is placed in the cavity 53d, and the sole edge members 52b and 52c are provided in the gaps between the molding half 53b and the sliding surface member 52a. Although figure 14B illustrates the molding half 53b over the molding half 53a, the molding halves 53a and 53b may be placed on a working table in such a manner as to upwardly direct the cavities 53c and 53d during the asemblage.

The molding halves 53a and 53b are opposed to each other as shown in figure 14B, and are assembled together. The mold 53 is enclosed in a flexible package 56, and is sealed therein. The inner space of the flexible package 56 is conencted to a vacuum source 57, and the air is evacuated from the inner space of the flexible package 56. As a result, the molding halves 53a and 53b are closely assembled inside the flexible package 56.

The flexible package 56 is, by way of example, formed of polyamide resin or from a lamination of polyamide resin/polyethylene, EVA resin/polyethylene, polyamide resin/ionomer or polyamide/EVA resin.

Higher vacuum promotes the impregnation of the melted matrix resin into the reinforcing fibers, and is desirable. In practical vacuum stage, the vacuum is developped at -755 mm/Hg inside the flexible package 56.

The mold 53 is heated to 100 - 120 degrees centigrade in vacuum for 35 minutes. The heat foams the elongated piece 54, and the foam outwardly presses the tubular fabric member 55b to the flexible matrix sheet 55a. The heat further melts the flexible matrix sheet 54a, and the tubular fabric member 55b is impregnated with the matrix resin. The foam further presses the tubular fabric member 55b impregnated with the matrix resin to expand, and presses the tubular fabric member 55b against the surface member 51a, the sliding surface member 52a and the sole edge members 52b and 52c. The foam is hardened, and is coverted to the core member 51c. The mold 53 is cooled in water at 15 degrees centigrade for 10 minutes. The tubular fabric member 55b impregnated with the matrix resin is hardened, and the reinforcing member 51b fills the gap between the core member 51c and the surface member 51a/the sliding surface member 52a/the sole edge members 52b and 52c as shown in figure 14D.

The sliding surface member 52a of high molecular polyethylene resin sets the limit on the highest temperature of the heat treatment, and the tubular fabric member 55b is expected to be impregnated with the matrix resin at not higher than 120 degrees centigrade. If the reinforcing member 51b is made from a prepreg, the reinforcing fibers may not sufficiently impregnated with the matrix resin at 120 degrees. However, the flexible matrix sheet 55a is melted and sufficiently impregnated into the reinforcing fibers by virtue of the laminated structure.

The mold 53 is taken out from the package 56, and the molding halves 53a and 53b are separated from one another. The ski shown in figure 13 is completed in the cavity 53c.

A press machine may presses the molding halves 53a and 53b to each other during the heat treatment. The pressing conditions are 2 kg/cm² x 2 minutes as an open pressure and 10 - 12 kg/cm² x ST as a main pressure. ST means time period for setting the resin.

The elongated piece 54 may be formed of more than one kind of foamable gum substance as similar to the first embodiment. Matrix resin sheets may be attached to the components of the upper/lower structures 51 and 52 instead of the flexible matrix sheet wound on the elongated piece 54.

As will be appreciated from the foregoing description, the elongated piece 54 of foamable gum substance internally produces the foam, and all the advantages of the first embodiment is also achieved by the second embodiment. The elongated piece 54 is inserted into the tubular fabric member 55b, and the relative position therebetween is hardly varied in the mold 53. Even if the elongated piece 54 is not a simple configuration, the tubular fabric member 55b follows the elongated piece 54, and topographically wound on the elongated piece 54. Therefore, the reinforcing fibers of the member 51b are oriented to designed direction or directions, and relatively small amount of reinforcing fibers imparts large strength to the ski. The sliding surface member 52a and the sole edge members 52b and 52c are hardly separated from the core member 51c, because they are integrated in the mold 53.

If a sleeve-shaped bias sheet made from glass fibers is used as the raw member for enhancing the torsional rigidity of the ski, liquid foamable substance hardly makes the bias sheet conformal to a complicated inner surface of the mold, because the pressure passes through the sleeve-shaped bias sheet to the complicated inner surface of the mold. However, the foamable gum substance effectively presses the sleeve-shaped bias sheet against the complicated inner surface of the mold, and causes the sleeve-shaped bias sheet to become conformal to the complicated inner surface of the mold. This results in large mechanical strength.

Although particular embodiments of the present invention have been shown and described, it will be obvious to those skilled in the art that various changes and modifications may be made without departing from the scope of the present invention.

For example, the process parameters are variable depending upon the substances of the components. The sliding surface member is usually formed of high molecular polyethylene resin, and the mold is heated to any temperature in so far as the sliding surface member is not deformed due to the heat.

Additional components may further be incorporated in the ski.

## Claims

1. A process of fabricating a ski comprising the steps of:
a) preparing a mold (29; 53) having a hollow space (29c/29d; 53c/53d) similar in configuration to said ski, a first member (21; 51a) for providing an outer surface of said ski, a second member (32; 55) for a reinforcing component (26; 51b), a third member (31; 54) of foamable gum substance, an expansible partition sheet (25) shorter in periphery than the periphery of said third member (31) and components (22/23a/23b; 52a/52b/52c) of a lower structure (28; 52) for producing sole edges and a sliding surface;
b) assembling said second member (32; 55) and said third member (31; 54) with said expansible partition sheet (25) being placed between said second member (32) and said third member (31) with said first member (21; 51a) and the components (22/23a/23b; 52a/52b/52c) of said lower structure (28; 52) in said hollow space;
c) foaming said foamable gum substance so as to expand in a space defined by said first member (21a; 51a) and said lower structure (28; 52);
d) setting the foam so as to fill said space with a core member (24; 51c) and said reinforcing component (26; 51b), thereby completing said ski; and
e) taking out said ski from said mold (29; 53).

2. The process as set forth in claim 1, in which said third member (32) of foamable gum substance has a plurality of sub-members (41a/41b; 42a/42b; 43a/43b/43c; 44a/44b; 45a/45b/45c) so as to produce a plurality of core sub-members different in compressive rigidity.

3. The process as set forth in claim 2, in which one of said plurality of sub-members (41a/41b; 42a/42b; 43a/43b/43c; 44a/44b; 45a/45b/45c) is differently regulated in expansion ratio from another of said plurality of sub-members (41a/41b; 42a/42b; 43a/43b/43c; 44a/44b; 45a/45b/45c).

4. The process as set forth in claim 3, in which said one of said plurality of sub-members (41a/41b; 42a/42b; 43a/43b/43c; 44a/44b; 45a/45b/45c) contains foaming agent different in content of said foamable gum substance from foaming agent of said another of said plurality of sub-members (41a/41b; 42a/42b; 43a/43b/43c; 44a/44b; 45a/45b/45c).

5. The process as set forth in claim 1, in which said second member (55) includes a tubular fabric member (55b) containing reinforcing fibers and a flexible sheet (55a) of matrix resin wound on said tubular fabric member (55b), and said third member 54 is inserted into an inner space of said tubular fabric member (55b).

6. The process as set forth in claim 1, in which said step (c) includes the sub-steps of
c-1) wrapping said mold (53) in a flexible package (56),
c-2) developing vacuum in said flexible package (56),
c-3) heating said mold (53).

7. The process as set forth in claim 6, in which said mold (53) is heated to a first temperature lower than a second temperature at which the component (52a) for said sliding surface is thermally deformed.

## Patentansprüche

1. Verfahren zur Herstellung eines Skis mit den Schritten:
a) Bereitstellung einer Form (29; 53) mit einem Hohlraum 29c/29d; 53c/53d) ähnlich der Gestalt des Skis, eines ersten Gliedes (21; 51a) zum Erhalt einer Außenfläche des Skis, eines zweiten Gliedes (32; 55) für eine Verstärkungskomponente (26; 51b), eines dritten Gliedes (31; 54) aus schäumbarer Gummisubstanz, eines dehnbaren Trennblattes (25) geringeren Umfangs als der Umfang des dritten Gliedes (31) sowie von Komponenten (22/23a/23b; 52a/52b/52c) einer unteren Struktur (28; 52) zur Herstellung einzelner Kanten sowie einer Gleitfläche;
b) Zusammensetzen des zweiten Gliedes (32; 55) und des dritten Gliedes (31; 54) unter Zwischenfügung des dehnbaren Trennblattes (25) zwischen das zweite Glied (32) und das dritte Glied (31) samt dem ersten Glied (21; 51a) und den Komponenten (22/23a/23b; 52a/52b/52c) der unteren Struktur (28; 52) in dem Hohlraum;
c) Schäumen der schäumbaren Gummisubstanz, so daß sie in einen Raum expandiert, der durch das erste Glied (21a; 51a) und die untere Struktur (28; 52) definiert wird;
d) Aushärten des Schaums, so daß er den Raum mit einem Kernglied (24; 51c) und die Verstärkungskomponente (26; 51b) ausfüllt, wodurch der Ski fertiggestellt wird, und
e) Entnehmen des Skis aus der Form (29; 53).

2. Verfahren nach Anspruch 1, worin das dritte Glied (32) aus schäumbarer Gummisubstanz eine Mehrzahl Unterglieder (41a/41b; 42a/42b; 43a/43b/43c; 44a/44b; 45a/45b/45c) aufweist, um eine Mehrzahl Kernunterglieder unterschiedlicher Drucksteifigkeit herzustellen.

3. Verfahren nach Anspruch 2, worin eines der Mehrzahl Unterglieder (41a/41b; 42a/42b; 43a/43b/43c; 44a/44b; 45a/45b/45c) auf ein gegenüber einem anderen der Mehrzahl Unterglieder (41a/41b; 42a/42b; 43a/43b/43c; 44a/44b; 45a/45b/45c) unterschiedliches Expansionsverhältnis eingestellt wird.

4. Verfahren nach Anspruch 3, worin dieses eine der Mehrzahl Unterglieder (41a/41b; 42a/42b; 43a/43b/43c; 44a/44b; 45a/45b/45c) einen anderen Anteil eines Schäummittels der schäumbaren Gummisubstanz gegenüber dem Schäummittel der anderen der Mehrzahl Unterglieder (41a/41b; 42a/42b; 43a/43b/43c; 44a/44b; 45a/45b/45c) aufweist.

5. Verfahren nach Anspruch 1, worin das zweite Glied (55) ein Verstärkungsfasern enthaltendes schlauchförmiges Stoffglied (55b) und ein um das schlauchförmige Stoffglied (55b) herumgewundenes flexibles Blatt (55a) aus Matrixharz aufweist und das dritte Glied (54) in einen Innenraum des schlauchförmigen Stoffgliedes (55b) eingesetzt wird.

6. Verfahren nach Anspruch 1, worin der Schritt c) die folgenden Unterschritte enthält:
c-1) Einpacken der Form (53) in eine flexible Packung (56),
c-2) Erzeugen eines Vakuums in der flexiblen Packung (56),
c-3) Erhitzen der Form (53).

7. Verfahren nach Anspruch 6, worin die Form (53) auf eine erste Temperatur erhitzt wird, die geringer ist als eine zweite Temperatur, bei welcher die Komponente (52a) für die Gleitfläche thermisch deformiert wird.

## Revendications

1. Procédé de fabrication d'un ski comportant les étapes consistant à :
a) préparer un moule (29 ; 53) ayant un espace creux (29c/29d ; 53c/53d) ayant une configuration similaire audit ski, un premier élément (21 ; 51a) pour fournir une surface extérieure dudit ski, un deuxième élément (32 ; 55) pour composant de renforcement (26 ; 51b), un troisième élément (31 ; 54) constitué d'une gomme pouvant être mise en mousse, une feuille de séparation dilatable (25) ayant une périphérie plus courte que la périphérie dudit troisième élément (31) et des composants (22/23a/23b ; 52a/52b/52c) d'une structure inférieure (28 ; 52) destinés à produire les bords de semelle et une surface de glissement,
b) assembler ledit deuxième élément (32 ; 55) et ledit troisième élément (31 ; 54), ladite feuille de séparation dilatable (25) étant placée entre ledit deuxième élément (32) et ledit troisième élément (31) avec ledit premier élément (21 ; 51a) et les constituants (22/23a/23b ; 52a/52b/52c) de ladite structure inférieure (28 ; 52), dans ledit espace creux,
c) transformer en mousse ladite gomme pouvant être mise en mousse de manière à la dilater dans un espace défini par ledit premier élément (21a ; 51a) et ladite structure inférieure (28 ; 52),
d) laisser durcir la mousse de manière à remplir ledit espace à l'aide d'un élément de coeur (24 ; 51c) et dudit composant de renforcement (26 ; 51b), en terminant ainsi ledit ski, et
e) enlever ledit ski dudit moule (29 ; 53).

2. Procédé selon la revendication 1, dans lequel ledit troisième élément (32) constitué d'une gomme pouvant être mise en mousse a plusieurs sous-éléments (41a/41b ; 42a/42b ; 43a/43b/43c ; 44a/44b ; 45a/45b/45c) de manière à produire plusieurs sous-éléments de coeur différents en ce qui concerne la rigidité en compression.

3. Procédé selon la revendication 2, dans lequel un desdits plusieurs sous-éléments (41a/41b ; 42a/42b ; 43a/43b/43c ; 44a/44b ; 45a/45b/45c) est régulé de manière différente en rapport de dilatation par rapport à un autre desdits plusieurs sous-éléments (41a/41b ; 42a/42b ; 43a/43b/43c ; 44a/44b ; 45a/45b/45c).

4. Procédé selon la revendication 3, dans lequel ledit premier desdits plusieurs sous-éléments (41a/41b ; 42a/42b ; 43a/43b/43c ; 44a/44b ; 45a/45b/45c) contient un agent moussant différent, dans le contenu de gomme pouvant être mise en mousse, d'un agent moussant d'un dit autre parmi lesdits plusieurs sous-éléments (41a/41b ; 42a/42b ; 43a/43b/43c ; 44a/44b ; 45a/45b/45c).

5. Procédé selon la revendication 1, dans lequel ledit deuxième élément (55) comporte un élément de tissu tubulaire (55b) contenant des fibres de renforcement et une feuille souple (55a) de résine de matrice enroulée sur ledit élément de tissu tubulaire (55b), et ledit troisième élément (54) est inséré dans un espace intérieur dudit élément de tissu tubulaire (55b).

6. Procédé selon la revendication 1, dans lequel ladite étape (c) comporte des sous-étapes consistant à :
c - 1) envelopper ledit moule (53) dans un emballage souple (56),
c - 2) développer un vide dans ledit emballage souple (56),
c - 3) chauffer ledit moule (53).

7. Procédé selon la revendication 6, dans lequel ledit moule (53) est chauffé à une première température plus basse qu'une seconde température à laquelle le composant (52a) de ladite surface de glissement est déformé thermiquement.
